

# United States Patent [19]

Sung et al.

[11] Patent Number: **4,676,917**

[45] Date of Patent: **Jun. 30, 1987**

[54] **RAILWAY DIESEL CRANKCASE LUBRICANT**

[75] Inventors: **Rodney L. Sung, Fishkill; Benjamin H. Zoleski, Beacon; Ronald L. O'Rourke, Hyde Park, all of N.Y.**

[73] Assignee: **Texaco Inc., White Plains, N.Y.**

[21] Appl. No.: **833,696**

[22] Filed: **Feb. 27, 1986**

[51] Int. Cl.<sup>4</sup> ..... **C10M 129/00; C10M 133/00**

[52] U.S. Cl. ..... **252/51.5 A; 252/51.5 R**

[58] Field of Search ..... **252/51.5 A, 51.5 R**

## [56] References Cited

### U.S. PATENT DOCUMENTS

|           |        |                 |       |            |
|-----------|--------|-----------------|-------|------------|
| 3,936,480 | 2/1976 | Demoures et al. | ..... | 252/51.5 A |
| 3,948,909 | 4/1976 | Okamoto         | ..... | 252/51.5 A |
| 4,048,080 | 9/1977 | Lee et al.      | ..... | 252/51.5 A |

|           |        |                  |       |            |
|-----------|--------|------------------|-------|------------|
| 4,374,741 | 2/1983 | Rieder           | ..... | 252/51.5 A |
| 4,427,562 | 1/1984 | Horodysky et al. | ..... | 252/51.5 A |
| 4,464,276 | 8/1984 | Sung et al.      | ..... | 252/51.5 A |
| 4,505,835 | 3/1985 | Sung et al.      | ..... | 252/51.5 A |
| 4,512,903 | 4/1985 | Schlicht         | ..... | 252/51.5 A |

Primary Examiner—William R. Dixon, Jr.

Assistant Examiner—Cynthia A. Prezlock

Attorney, Agent, or Firm—Robert A. Kulason; James J. O'Loughlin; Vincent A. Mallare

## [57] ABSTRACT

A crankcase lubricating oil composition for railway diesel engines, containing a mineral lubricating oil, an overbased calcium alkylphenolate and an alkyaryl sulfonate oxidation and corrosion inhibiting amount of a reaction product of polyoxyisopropylene diamine, dibasic acid anhydride and polyalkylene polyamine.

**9 Claims, No Drawings**





analysis) may be represented by the following flow process diagram.

In the process illustrated below, initially, maleic anhydride (A) is reacted with polyoxoisopropylenediamine (B) to form maleamic acid (C). Then, the maleamic acid (C) is reacted with a polyalkylene polyamine (D) to form the condensate product (E) of polyoxoisopropylenediamine, maleic anhydride, and polyalkylene polyamine. Accordingly, the condensate product (E) is recovered.

of the polyoxoisopropylenediamine JEFFAMINE D-400 at 100° C. for 2 hours. JEFFAMINE D-400 is a polyoxoisopropylenediamine of approximate molecular weight 5.9 having the general formula:



10 where x has an approximate value of 2 to 50. The mix-



wherein x is a numeral of about 5.0, n is about 0 to about 4, and m is about 0 to about 2.

The prepared reaction product, i.e., condensate product may be added to a fuel in a minor deposit-inhibiting amount of about 0.001 to about 0.1 weight percent, and preferably from about 0.01 to about 0.1 weight percent of the reaction product.

The advantages and features of the present invention

ture was thereafter cooled to about 60° C., and 25.8 parts of diethylene triamine were added. The new mixture was then reacted at about 100° C. for 2 hours to produce the final reaction product. The reaction product was filtered and stripped of the remaining solvent under a vacuum. The final reaction product structure (as evidenced by elemental analysis, IR analysis, and NMR analysis) was as previously described.



will be more apparent from the Examples below. The following examples illustrate the preferred method of preparing the reaction product of the instant invention. It will be understood that the following examples are merely illustrative and are not meant to limit the invention in any way. In the example, all parts are parts by weight unless otherwise specified.

The Jeffamine D series are manufactured and marketed by Texaco Chemical Company of Houston, Tex.

#### EXAMPLE I

A reaction product was formed by reacting 245 parts of maleic anhydride, 260 parts of xylene, and 102.7 parts

60 ps where x has a value from about 20 to 50 depending upon the particular JEFFAMINE D reactant employed, and n has a value from about 0 to 4 and m has a value from about 0 to 2, depending upon the particular polyalkylene polyamine reactant employed.

The anti-oxidation and anti-corrosion agents are provided in the examples below.

65 IN examples II through VII, the same procedure is used as that in Example I except for the amount of polyoxoisopropylenediamine and polyalkylene polyamine. Thus, for each example, the amount of polyether

amine and polyalkylene polyamine are provided below with the structure of the condensate product.

### EXAMPLE II

Amount of Jeffamine D-400: 410.7 parts.  
Amount of Diethylene Triamine: 103 parts.

5

Amount of Jeffamine D-2000: 1968.4 parts.  
Amount of Triethylene Tetramine: 145 parts.



(where  $x$  is 5.58).

15



### EXAMPLE III

Amount of Jeffamine D-400: 410.7 parts.  
Amount of triethylene Tetramine: 145 parts.



(where  $x$  is 5.58).



#### EXAMPLE IV

Amount of Jeffamine D-230: 114.8 parts.  
Amount of Diethylene Triamine: 103 parts.

20 (where  $x$  is 33).

Preferred components for the lubricating oil of the invention are those which are effective in a range from



(where  $x$  is 2–3).

### EXAMPLE V

Amount of Jeffamine D-2000: 1968.4 parts.  
Amount of Diethylene Triamine: 103 parts.

about 0.1 to 5 weight percent based on the total lubricating oil composition. However, it is preferred to employ from about 0.5 to 2 weight percent of the derivative based on the weight of the lubricating oil with the most preferred concentration ranging from about 0.75 to 1.5



(where  $x$  is 33).

### EXAMPLE VI

Amount of Jeffamine D-230: 114.8 parts.  
Amount of Triethylene Tetramine: 145 parts.

55 weight percent.

weight percent.

The following Examples illustrate the best mode of making and using the oxidation and corrosion reducing additive component of the railway diesel oil composition of the invention.



(where  $x$  is 2-3)

## OIL OXIDATION TEST

The test method involves bubbling 5 liters of oxygen per hour through 300 mls. of test oil composition at 285° F. in which there is immersed a 1×3×0.06 inch steel backed copper-lead test specimen cut from bearing stock. The viscosity of the test oil is measured before and after the 144 hour test period and greater the difference in viscosity the greater the oxidative deterioration of the instant invention. In addition, the test specimen is weighed before and after the test period and the greater the weight loss of test specimen the greater the corrosion deterioration of the test formulation. Further, the larger the amount of copper, iron and lead moieties found in the oil after test the greater the oxidative corrosion deterioration thereof.

The representative Formulations A, B, F, G and comparative Formulations C, D and F and their oxidation test results are reported below in Table II:

TABLE II

| Oil Code                                                          | OIL OXIDATION TEST <sup>3</sup> |        |
|-------------------------------------------------------------------|---------------------------------|--------|
|                                                                   | A                               | B      |
| <u>Composition, wt %</u>                                          |                                 |        |
| Overbased                                                         | 4.10                            | 4.10   |
| [An alkaryl sulfonate/phenate <sup>(1)</sup> ]                    |                                 |        |
| Ca salt of polyisobutylene phenol-aldehyde-amine reaction solvent | 1.46                            | 1.46   |
| Polyisobutylene                                                   | 0.44                            | 0.44   |
| Branched alkyl (C <sub>16</sub> ) phenol                          | 0.88                            | 0.88   |
| Chlorowax                                                         | 0.15                            | 0.15   |
| SNO-320                                                           | 19.64                           | 20.14  |
| SNO-850                                                           | 30.02                           | 30.52  |
| 75/80 Pale Oil                                                    | 37.31                           | 37.31  |
| Low Quality                                                       | 5.00                            | 5.00   |
| Marine Diesel fuel <sup>(2)</sup>                                 |                                 |        |
| Experimental Anti-oxidation                                       | 1.0                             | —      |
| Anti-corrosion Additive I <sup>(3)</sup>                          |                                 |        |
| <u>Test Results</u>                                               |                                 |        |
| Wt Loss-gm                                                        | 0.0079                          | 0.2574 |
| Viscosity increase, %                                             | 27.6                            | 82.0   |

(1)The ratio of sulfonate to phenate is 1:1.

(2)Low quality marine diesel fuel (Bunker-C); see Attachment I below for specifications.

(3)Reaction product of Jeffamine D-400, maleic anhydride & diethylene triamine.

## ATTACHMENT I

|                                    |       |
|------------------------------------|-------|
| Density, g/ml 15° C.               | 0.962 |
| Viscosity, CST at 50° C.           | 173   |
| Water content, 0/0 V/V             | 0.0   |
| Conradson: Carbon residue, 0/0 M/M | 12.7  |
| Sulphur: 0/0 M/M                   | 1.47  |
| Ash, 0/0 M/M                       | 0.06  |
| Vandium: MG/KG                     | 30    |
| Sodium, MG/KG                      | 120—  |
| Allminium, MG/KG                   | 16    |
| Silicon, MG/KG                     | 38    |
| Compatibility with MGO             | No. 1 |
| Calc. lower heat value, MJ/KG      | 40.63 |

We claim:

1. A railway diesel crankcase lubricant composition comprising a diesel lubricating oil and from about 0.25 to 2.0 weight percent of minor amount of oxidation and corrosion inhibiting agent, the reaction product of a polyoxyisopropylene diamine, dibasic acid anhydride and polyalkylene polyamine wherein:

(i) reacting a dibasic acid anhydride with a polyoxyisopropylenediamine



where x is a numeral of about 2 to about 50, thereby forming a maleamic acid;

(ii) reacting said maleamic acid with a polyalkylene polyamine, thereby forming a condensate product and;

(iii) recovering said condensate product.

2. The railway diesel crankcase lubricant composition of claim 1, wherein said polyoxyisopropylenediamine has a molecular weight  $\bar{M}_n$  ranging from about 230 to about 2000.

3. The railway diesel crankcase lubricant composition of claim 1, wherein said polyoxyisopropylenediamine, x is a numeral of about 2 to about 33.

4. The railway diesel crankcase lubricant composition of claim 1, wherein said dibasic acid anhydride has the formula



where R is H, CH<sub>3</sub>— or C<sub>2</sub>H<sub>5</sub>—.

5. The railway diesel crankcase lubricant composition of claim 1, wherein said polyamine has the formula



where n is a numeral of about 0 to about 4 and m is a numeral of about 0 to about 2.

6. The railway diesel crankcase lubricant composition of claim 1, wherein the minor anti-oxidation inhibiting amount ranges from about 0.25 to about 2.0 weight percent of the said reaction product.

7. The railway diesel crankcase lubricant composition of claim 6, wherein the minor anti-oxidation and anti-corrosion amount is about 0.25 to about 2.0 weight percent of said reaction product.

8. A railway diesel crankcase lubricant composition comprising:

(a) a major portion of a liquid naphthenic mineral oil having a viscosity of 300 at 100° F. paraffinic oil and naphthene mineral oil of 75-80 viscosity at 210° F.;

(b) a minor amount, as a deposit-inhibiting additive of a condensate product of the process comprising:

(i) reacting a polyoxyisopropylenediamine



where x is a numeral of about 2 to about 50, with a dibasic acid anhydride



where R is H,  $\text{CH}_3$ — or  $\text{C}_2\text{H}_5$ —, thereby forming a maleamic acid; 10

(ii) reacting said maleamic acid with a polyalkylene polyamine



5

where  $n$  is about 0 to about 4 and  $m$  is about 0 to about 2, thereby forming a condensate product



where  $x$  is about 2 to about 50;  $n$  is about 0 to about 4; and  $m$  is about 0 to about 2; and

(iii) recovering said condensate product.

9. A diesel crankcase lubricant composition:  
(a) a major portion of a liquid having a naphthenic

15

mineral oil, naphthenic mineral oil of 75-80 viscosity at 210° F. and

(b) about 1 wt.% of a anti-oxidation and corrosion-inhibiting condensate product of the process comprising:

(i) reacting a polyoxvisopropylendiamine



where x is a numeral of about 2 to about 50 with maleic anhydride, thereby forming a maleamic acid



(ii) reacting said maleamic acid with diethylene triamine, thereby forming a condensate product



and  
(iii) recovering said condensate product.

mineral oil of viscosity of 300 at 100° F., paraffinic

4

58

5

61

6